

## [54] CORONA DISCHARGE TREATMENT OF FOAM FIBRILLATED WEBS

[75] Inventor: Gary L. Driscoll, Boothwyn, Pa.

[73] Assignee: Sun Research and Development Co., Philadelphia, Pa.

[22] Filed: Jan. 2, 1973

[21] Appl. No.: 320,353

[52] U.S. Cl. .... 264/22; 156/79; 156/229; 156/272; 264/54; 264/210 R; 264/DIG. 5; 264/DIG. 8; 428/310

[51] Int. Cl.<sup>2</sup> .... B29D 27/00; B29C 25/00; H05B 7/16

[58] Field of Search .... 264/51, 53, 54, DIG. 8, 264/22, 210 R; 156/152, 272, 79, 229, 307, 316; 117/93.1, 47 A; 161/72; 428/310

## [56] References Cited

## UNITED STATES PATENTS

|           |         |                       |               |
|-----------|---------|-----------------------|---------------|
| 2,859,480 | 11/1958 | Berthold et al. ....  | 156/272 X     |
| 2,923,964 | 2/1960  | Plonsky.....          | 156/272 X     |
| 2,935,418 | 5/1960  | Berthold et al. ....  | 117/93.1 CD X |
| 3,067,179 | 12/1962 | Ramika.....           | 117/47 A X    |
| 3,099,572 | 7/1973  | Rion et al. ....      | 117/47 A      |
| 3,111,418 | 11/1963 | Gilbert et al. ....   | 117/47 A X    |
| 3,169,899 | 2/1965  | Steuber.....          | 161/72        |
| 3,391,044 | 7/1968  | Kaghan et al. ....    | 156/272       |
| 3,539,666 | 11/1970 | Schirmer.....         | 264/DIG. 8    |
| 3,562,369 | 2/1971  | Chopra et al. ....    | 264/DIG. 8    |
| 3,576,931 | 4/1971  | Chopra et al. ....    | 264/DIG. 8    |
| 3,661,671 | 5/1972  | Katagiri et al. ....  | 156/272       |
| 3,754,117 | 8/1973  | Walter.....           | 156/272 X     |
| 3,860,369 | 1/1975  | Brethauer et al. .... | 264/22 X      |

## FOREIGN PATENTS OR APPLICATIONS

|           |         |                     |            |
|-----------|---------|---------------------|------------|
| 1,192,132 | 5/1970  | United Kingdom..... | 264/DIG. 8 |
| 1,171,971 | 11/1969 | United Kingdom..... | 264/DIG. 8 |

## OTHER PUBLICATIONS

"The Naming and Indexing of Chemical Compounds

From Chemical Abstracts," Introduction to the subject index of vol. 56, Washington, D. C., American Chemical Society, 1962, pp. 12N-15N; 37N-40N; 44N; 45N; 87N-89; 94N-95N.

"The Condensed Chemical Dictionary," Eighth Edition, revised by Gessner G. Hawley, New York, Van Nostrand Reinhold, 1971, p. 87.

Muus, Laurits T., N. Gerard McCrum, and Frank C. McGrew, "On The Relationship of Physical Properties to Structure in Linear Polymers of Ethylene and Propylene," In SPE Journal, May 1959, pp. 368-372.

Sharpe, Louis H. and Harold Schonhorn, "Surface Energetics, Adhesion and Adhesive Joints," In contact angle, wettability and adhesions the Kendall Award Symposium honoring William A. Zisman sponsored by the division of Colloid and Surface Chemistry at the 144th meeting of the American Chemical Society, Los Angles, Calif., Apr. 2-3, 1963, Washington, D.C., American Chemical Society, 1964, pp. 189-201, (advances in Chemistry Series 43).

McLaren, A. D.; T. T. Li; Robert Rager and H. Mark, "Adhesion IV, The Meaning of Tack Temperature," In Journal of Polymer Science, vol. VII, No. 5, pp. 463-421 (1951).

Primary Examiner—Philip Anderson

Attorney, Agent, or Firm—J. Edward Hess; Donald R. Johnson; Anthony Potts, Jr.

[57]

## ABSTRACT

Non-woven fabrics are produced from polyolefin foam fibrillated webs. The webs are treated with corona discharge to improve the adhesion thereof when they are laminated under heat and pressure to form a non-woven fabric.

1 Claim, 2 Drawing Figures



Fig. 1



Fig. 2



## CORONA DISCHARGE TREATMENT OF FOAM FIBRILLATED WEBS

### BACKGROUND OF THE INVENTION

In the past there has been considerable effort to find a way of forming fabric-like materials by means other than weaving or knitting, due to the expense involved therein. Weaving fabrics is a particularly expensive operation, and especially so when the woven material is made from fiber slivers. Woven slit film eliminates the carding or garneting of fibers, but still involves the expensive weaving operation. Needle punching of layers of fibrillated films is used for some purposes but for many purposes the layers are not sufficiently unitized. Bonding of polyolefin fibrillated webs has generally not been used because of insufficient adhesion of the webs.

### SUMMARY OF THE INVENTION

The present invention relates to surface treating polyolefin foam fibrillated webs so as to improve their adhesion to each other when they are assembled to form a non-woven fabric. The web is formed of a polymer of one or more  $\alpha$ -olefins containing from 2 to 10 carbon atoms. Examples of such  $\alpha$ -olefins include polyethylene, polypropylene, copolymers of ethylene and propylene or blends thereof, polybutene-1 and polymethylpentene-1. Generally the web will contain at least 70 wt. % of the poly  $\alpha$ -olefin. Thus the web may contain up to 30 wt. % of another polymer such as polystyrene, ethylene-vinyl acetate copolymer, acrylic polymers, etc. The webs are treated with a corona discharge having an intensity of from 1 watt-minute/ft<sup>2</sup> to 75 watt-minutes/ft<sup>2</sup>, at from 25° to 150°C. The webs are assembled into a plurality of layers by any suitable means such simply unrolling some webs onto a carrier belt and cross-lapping some other layers to provide strength across the machine direction of the final non-woven fabric. The assembled layers are finally laminated together using a combination of heat and pressure. An adhesive may be used if desired but its presence is not required.

### DESCRIPTION OF THE DRAWINGS

FIG. 1 is a schematic side view of the foam extrusion and fibrillation apparatus.

FIG. 2 is a schematic side view of the laminating apparatus.

In FIG. 1 the polyolefin is fed to hopper 1 of feed meterer 2, along with whatever blowing agent is required. The polyolefin is fed at a controlled rate from feed meterer 2 to the feed hopper 3 of extruder 4 as free falling pellets 5. Extruder 4 is equipped with a slit die 6, the slit of which is offset from the extruder feed-port so as to create sufficient back pressure to provide for a uniform feed rate across the width of the die. The extrudate is taken up and attenuated by a first pair of nip rolls 7,7'. As the extrudate leaves the die lips it is air quenched by means of an air quench manifold 8 which is provided with ports directed at the extrudate. A hood 9 is provided to remove the gaseous blowing agent from the atmosphere since the blowing agent may contain noxious fumes. First pair of nip rolls 7,7' are operated at a surface rate speed of from 2 to 25 times the linear rate at which the polyolefin is supplied to the lips of die 6 by extruder 4. This serves to break the foam bubbles within die 6 as they approach the lips of die 6 or immediately as they leave die 6, whereby a foam fibrillated

web 10 is formed. The foam fibrillated web 10 is passed over heated shoe 11, and drawn by a second pair of nip rolls 12,12'. Generally second pair of nip rolls 12,12' are driven at a surface speed rate of from 2 to 10 times the surface speed rate of first pair of nip rolls 7,7' to orient and thereby strengthen foam fibrillated web 10. The thus oriented foam fibrillated web 10 is then passed between corona discharge platens 13 and 14 to treat the surface of the foam fibrillated web 10. The foam fibrillated web 10 is then passed under idler roller 15 and is taken up on take-up reel 16.

In FIG. 2 a reel 17 supplies foam fibrillated web 18 to carrier belt 19. An additional layer of foam fibrillated web 20 is fed from reel 21, supported overhead by means not shown, to lapper 22. Lapper 22 contains a pair of driven nip rolls mounted in a carriage. The nip rolls feed the foam fibrillated web 20 onto first foam fibrillated web 18. This results in the foam fibrillated web being laid down at a 45° angle to the machine direction in a double thickness. Another reel 23 supplies foam fibrillated web 24 to second lapper 25 onto lapped foam fibrillated web 20 to form two layers of foam fibrillated web 24 disposed at 45° to the machine direction. A final layer of foam fibrillated web 26 is fed from reel 27 onto foam fibrillated web 24. The entire lay-up of foam fibrillated webs is then removed by carrier belt 19 and passed through heated laminating rolls 28,28'. If desired adhesive may be applied to the lay-up of foam fibrillated webs by means of sprayers 29 and 30. The laminated foam fibrillated webs are then taken up on take-up reel 31.

### DETAILED DESCRIPTION

In preparing the foam fibrillated webs of the present invention several extrusion and drawing techniques may be employed. The drawings show the preferred technique. However, for instance the extruder may be fed by any suitable means including manually from sacks of polyolefin resin. A slit die has been shown and has been found most convenient for forming relatively narrow width webs of from say 6 inches to 5 feet. For wider webs of say 3 to 20 feet an annular die has obvious advantages. When using such an annular die the web is drawn over a mandrel to maintain or slightly increase its circumference during orientation.

The extruder used may be equipped with a port to inject the blowing agent. If this is done, various blowing agents may be used such as the Freons, methylene chloride, nitrogen, carbon dioxide, etc. If the extruder is not equipped with a port to inject the blowing agent, the blowing agent is fed into the extruder along with the polyolefin. While this can be done by coating the polyolefin pellets with a low boiling liquid such as pentane which becomes a gas at the elevated temperature in the extruder, it is preferred to use a solid blowing agent. Such solid blowing agent is physically or chemically decomposed to form a gas in the extruder. Exemplary solid blowing agents include but are not limited to azobisformamide, azobisisobutyronitrile, diazoamino-benzene, 4,4'-oxybis(benzenesulfonylhydrazide), benzenesulfonylhydrazide, N,N'-dinitrosopentamethylene-tetramine, trihydrazino-symtriazine, p,p'-oxybis(benzenesulfonylsemicarbazide)-4-nitrobenzene sulfonic acid hydrazide, beta-naphthalene sulfonic acid hydrazide, diphenyl-4,4'-di(sulfonylazide) and mixtures of materials such as sodium bicarbonate with a solid acid such as tartaric acid. The amount of blowing agent to be used in the process generally is in the range

of from 0.1 to 20 wt % of the polyolefin being extruded with from 0.5 to 5.0 wt % being the preferred range.

The polyolefin used generally will have a melt index of below 30 g. Almost any commercial polyolefin plastic is suitable whether it be molding, film or fiber grade.

As the polyolefin is extruded it is taken up by a take-up means such as a first pair of nip rolls and attenuated about 2 to 25 times. This attenuation serves to cause the foam bubbles forming within the die to break as the blend approaches the die lips resulting in a network or web of intertwined and connected fibrils. The temperature of the polyolefin is generally maintained at from 120° to 315°C. From 190° to 230°C is the preferred range for polypropylene. From 150° to 200°C is the preferred range for polyethylene. As the polyolefin leaves the die lips it is quenched by any suitable means such as an air quench which serves to insure that the polyolefin is solidified to develop adequate strength to pull it away from the die which occurs below about 150°C in the case of polypropylene and below about 110°C in the case of polyethylene. This causes the foam bubbles which were forming as the pressure imposed on the polyolefin drops as the polyolefin approaches the die lips to rupture and form fibrils rather than merely to expand into larger bubbles. After this foam fibrillated web has been formed it is then stretched to orient the polyolefin which makes up the individual fibrils which in turn make up the web, thereby strengthening the web. Normally this stretching is from 2 to 10 times but in any case is below where breakage of the web occurs. Generally the webs are stretched at a moderately elevated temperature.

The webs are then subjected to treatment with corona discharge. This treatment is generally carried out at a moderate temperature of from 25° to 150°C. Generally the amount of corona discharge applied is in the range of from 1 to 75 watt-minutes per square foot of web. It is surprising that corona discharge is operable on these webs because when it is applied to film any pin holes, etc. cause arcing and an unsatisfactory operation.

This treatment serves to markedly improve the bonding of the webs together. This improvement is observed both when the webs are laminated by heat and pressure and when an adhesive is used.

The adhesive can be a liquid which is sprayed, doctor or otherwise applied to whatever webs are to be assembled into a non-woven fabric. Any thermoplastic adhesive which softens in the range of from 100° to 170°C can be used or cross-linking formulations can be applied. The commercially available ethylene-vinyl acetate copolymer emulsions are particularly satisfactory adhesives for the purpose.

Generally the die used to extrude the webs has an opening of from 15 to 25 mils in the thickness direction which results in the final oriented foam fibrillated webs weighing from 0.2 to 0.8 ounces per square yard. Generally the final non-woven fabric will contain from 3 to 20 layers of web. For most uses such as industrial bagging, primary carpet backing, secondary carpet backing, wallpaper, upholstery backing, etc. from 5 to 10 layers of web are used and the non-woven fabric product has a weight of from 2.5 to 10 ounces per square yard. There are a plurality of ways in which the layers of webs can be assembled. Often the way in which the webs are assembled is dependent on the use to which the non-woven product is to be put. Usually this involves 3-4 layers in the machine direction and 2-6

layers at an angle thereto. However the webs can be run through a tenter frame to increase their width 2 to 6 times which imparts a biaxial disposition to the direction of the individual fibrils within the web, in which case all of the webs can be laid down in the machine direction and laminated.

For individual laminates of from about 6 inches square up to about 4 × 8 ft. a press can be used to laminate the foam fibrillated webs together. Generally such a press is operated at from 10 to 500 p.s.i. and at 90° to 150°C. For long rolls of the non-woven product heated pressure rolls are used. Generally these are heated metal rolls, preferably steel rolls or coated steel rolls operated at from 2 to 200 lbs. per lineal inch pressure, from 90° to 150°C and the material being laminated is fed at a rate of from 10 to 300 feet per minute. The hand, appearance, porosity and other physical characteristics of the non-woven fabric product can be varied considerably by varying the severity of the laminating conditions within the parameters set forth above. Further these characteristics of the product non-woven fabric can be varied by using embossed or textured laminating rolls. If one (or if desired both) laminating rolls (or one or both surfaces of a press if such is being used) are covered with burlap or a screen of the appropriate size mesh a non-woven fabric which looks like burlap can readily be obtained. This is a distinct advantage over most other non-woven fabrics or even woven slit film in the production of secondary carpet backing where aesthetics are important and where burlap, which is now in short supply, has been the traditional material used.

#### EXAMPLES

35 A Killian one inch extruder having a 24 to 1 length to diameter ratio screw is equipped with an eight inch wide slit die having a 20 mil thick opening. The slit is offset from the screw by 10 inches and extrudes in a direction parallel to the direction of the extruder barrel. The extruder hopper is hand filled with a blend of polypropylene having a melt index of 10, and 1 wt. % of Celogen AZ (azodicarbonamide). The extruder barrel is maintained at 175° to 230°C from the feed end to the die end and the die at 230°C. The screw is operated at 25 rpm. Immediately adjacent the die lips is an air quench which is a pair of 0.5 inch diameter pipes one located above the die lips and the other below the die lips containing air under 80 p.s.i. pressure. Each pipe contains a row of 0.030 inch diameter holes 0.125 inch apart directed at the die lips. The extrudate is withdrawn from the die lips by a first pair of five inch diameter nip rolls 8 inches in width driven at a surface speed of 15 ft./min. to form a foam fibrillated web. These rolls comprise a driven rubber covered roll and a stainless steel idler roll. The foam fibrillated web is then passed over a heated shoe eight inches wide and 36 inches long. The shoe is slightly arched in shape so as to maintain the foam fibrillated web in intimate contact with it. The shoe is maintained at 135°C. The foam fibrillated web is then passed between a second pair of nip rolls identical to the first pair of nip rolls operated at a surface speed of 45 ft./min. The web is passed between a grounded 12 × 14 inch aluminum plate covered with 30 mils of poly(ethylene terephthalate) and a high voltage electrode which is a  $\frac{3}{8} \times 1 \times 12$  inch aluminum bar one-eighth inch from the grounded electrode at a rate of 45 ft./minute. The high voltage electrode is connected to a generator supplying 450 watts of power at

2000 Hz frequency and at about 15,000 volts. This gives a 10 watt-minutes/ft.<sup>2</sup> treatment. The web is then taken up on a take-up reel. The web is cut into six 6-inch squares which are laid up by hand with three layers in one direction and three layers at right angles thereto. The six layers of web are then laminated by pressing at 150°C and 10,000 pounds total pressure for 3 minutes. Tensile strips 6 inches long and one inch wide are cut at 45° from the direction of the webs. These strips exhibited a strength of 0.05 g/denier versus controls which were not surface treated of <0.01 g/denier. This strength test is directly dependent on bond strength since the pairs of jaws of the tester are spaced 3 inches apart and since the fibrils within the individual webs are at a 45° angle to the pulling direction none of them are being pulled by both pairs of jaws.

The invention claimed is:

1. A process of producing a foam fibrillated fibrous web comprising extruding a resinous composition at least 70 weight percent of which is a poly  $\alpha$ -olefin, and a gaseous material mixed with said polyolefin from a die into a zone of reduced pressure to produce an extrudate, withdrawing said extrudate from said die by a first take-up means at a linear rate from 2 to 25 times the linear rate at which said polyolefin reaches the die lips to form a foam fibrillated web, stretching said foam fibrillated web from 2 to 10 times in the machine direction, and surface treating the stretched foam fibrillated web with a corona discharge at an intensity of from 1 to 75 watt-minutes per square foot at about 20 to about 150°C whereby the fibrous web has improved adhesion ability with itself.

\* \* \* \* \*

20

25

30

35

40

45

50

55

60

65